

## 1

3,016,338

## ELECTROLYTIC RECORDING PAPER

Gerald Mandel, Flushing, N.Y., assignor, by mesne assignments, to Hogan Faximile Corporation, a corporation of Delaware  
No Drawing. Filed Aug. 4, 1958, Ser. No. 753,075  
13 Claims. (Cl. 204—2)

This invention relates to the art of electrically markable recording media and particularly concerns an improved electrolytic recording paper.

Recording paper of the electrolytic type is marked by disposing the paper between electrodes consisting of a positive metal anode and a negative cathode. The paper is impregnated with an electrolytic solution containing a marking compound. This compound is capable of reacting with ions supplied by the anode to form a colored mark wherever the anode contacts the paper.

Recording paper employed for facsimile recording purposes must meet certain important requirements. The paper must have the ability to produce marks having a density which is a function (preferably linear) of the current passed through the paper. The paper must remain active and resist discoloration when stored for extended periods of time. Recorded marks should be stable when the paper is exposed to ambient conditions of light and air. The active ingredients in the impregnant of the paper must avoid discoloration of or diffusion to adjacent sheets of marked or unmarked paper of the same or different types.

It has been known heretofore that an electrolytically markable paper could be made with a marking compound that formed a dark complex ion with the metal ions released by the anode. The marks thus formed have generally been described as colored lakes. While recording papers made with such compounds are generally satisfactory it has been noted that they are subject to several disadvantages. There has been noted a tendency to bleach of marked portions of paper when the paper is rolled or folded in a wet condition. A transfer effect has also been noted. This effect appears when dry paper in marked or unmarked state containing lake-forming marking compounds causes discoloration of adjacent sheets of paper which do not contain any marking compound.

The present invention involves a high speed precipitation reaction to provide a superior type of electrolytic recording paper. In this type of paper there is provided an impregnant containing a compound which forms a precipitant in aqueous solution as a reaction product with the metal ions. In the present invention, the current functions only to electrodeposit metal ions into the paper and no part of the ionizing electric current is required to effect precipitation of the reaction product.

According to the present invention there is provided an electrolytic recording paper which displays excellent stability in storage. It produces clearly defined marks which are stable and do not fade on standing. The marks do not transfer or bleach. Unmarked paper in a moist state retains its marking characteristics.

Recording papers embodying the present invention contain chromotropic acid as a marking agent or marking compound. This compound is also known as 4,5-dihydroxy-2,7-naphthalene-disulfonic acid disodium salt. The marking compound forms a light colored yellow or green aqueous solution and forms a dark colored insoluble compound with ions of a metal anode so that the insoluble compound precipitates out of the solution.

Satisfactory results are obtained with metal anodes such as stainless steel containing iron which result in emerald green marks, or copper anodes which result in

## 2

red-brown marks, or titanium anodes which produce brick red marks.

Chromotropic acid is a colorless crystalline compound which wholly dissolves in an aqueous solution having a properly adjusted pH so that upon impregnation of white porous paper with a solution which has been rendered properly electroconductive there is obtained an electrically markable recording paper. Upon application of a suitable metal anode to the impregnated paper and applying an electric current, the metal electrodeposits into the impregnant in the paper and a colored precipitant is formed. A suitable electrolyte must be added to the weakly acid impregnant to render it properly electrically conductive for marking to occur.

It has been discovered that addition of chromotropic acid to a formulation containing tannic acid as the marking compound in an electrolytic recording paper produces several desirable and unusual results. Normally electrolytic recording paper containing tannic acid produces marks having a purple tone or cast. If the marking current is increased this purple color becomes most pronounced. In many recording applications it is desired that the resulting marks be black and free from any purple or other off-black tone. Addition of chromotropic acid to the formulation has the effect of preventing off-black marking to result in dark black marks. It has also been noted that in tannic acid marking papers it is necessary to increase the marking current to increase the darkness of the recorded marks. Addition of chromotropic acid to the formulation results in production of darker and blacker marks without requiring an increase in the marking current.

Typical formulations of impregnants of paper which can be used are as follows:

|    |                      |                                                                               |
|----|----------------------|-------------------------------------------------------------------------------|
|    |                      | I                                                                             |
| 35 | Chromotropic acid    | grams 5                                                                       |
|    | Potassium nitrate    | do 10                                                                         |
|    | Water                | cc 100                                                                        |
| 40 |                      |                                                                               |
|    |                      | II                                                                            |
|    | Chromotropic acid    | 2 grams.                                                                      |
|    | Potassium nitrate    | 10 grams.                                                                     |
|    | Tannic acid          | 5 grams.                                                                      |
|    | Water                | 100 cc.                                                                       |
| 45 | Sulfuric acid (6 N)  | Sufficient to adjust the pH of the solution for optimum marking (about 1.25). |
|    |                      | III                                                                           |
| 50 | Chromotropic acid    | 2 grams.                                                                      |
|    | Potassium nitrate    | 10 grams.                                                                     |
|    | Tannic acid          | 5 grams.                                                                      |
|    | Monosodium phosphate | 0.1 gram.                                                                     |
|    | Sodium bitartrate    | 0.25 gram.                                                                    |
| 55 | Thiourea             | 0.15 gram.                                                                    |
|    | Water                | 100 cc.                                                                       |
|    | Sulfuric acid (6 N)  | Sufficient to adjust the pH of the solution for optimum marking (about 1.25). |
| 60 |                      |                                                                               |

The potassium nitrate serves as an electrolyte to adjust the electrical conductivity of the solution. Other inorganic salts may be used for this purpose such as NaCl, KCl, NaNO<sub>3</sub>, etc. The monosodium phosphate and sodium bitartrate provide phosphate and tartrate ions which act to prevent fringing or spreading of the recorded marks. Sources of citrate, oxalate, and maleate ions can be used for a similar purpose. Thiourea acts as a stabilizer to prevent discoloration of the impregnated recording paper in a marked and unmarked state.

Instead of sulphuric acid, hydrochloric acid, nitric acid, or other acids may be used. Since the acid is an elec-

troyte the quantity of salt electrolyte necessary will depend on the acid concentration. The pH adjustment selected, i.e., the quantity of acid used, will depend on the depth of colored mark desired and type of metal anode used. A pH of about 1.25 has been found to result in satisfactory marking. The acid used must not adversely affect the precipitation reaction. If the impregnant is made too strongly acid, the recorded marks tend to fade and the porous paper support may be attacked and weakened by the acid content. If the impregnant is made too basic, the resulting marks assume a red or purple cast.

To prepare the recording paper with any of the substances mentioned above, the marking compound and electrolyte are dissolved in water, or acid. White, porous paper having a high wet strength is then immersed in the solution. Upon removal the paper is ready for being marked between electrodes to which a direct current is applied between a cathode and anode applied in contact with opposite sides of the paper. The anode electrode must contain a metal, such as iron, which will electrodeposit into the impregnant during the application of electric current through the paper. The metal must be one which will form a dark colored precipitant with the marking compound.

For use in recording, the impregnated paper can be marked in a facsimile recorder of the type described in Patent 2,575,959 issued to J. V. L. Hogan.

Certain specific combinations and compositions have been given by way of example. However, it will now be apparent to those skilled in the art that various modifications and changes may be made within the spirit and scope of the invention as defined in the appended claims.

What is claimed is:

1. An electrolytic recording medium comprising an impregnated sheet containing as a marking compound chromotropic acid in an electrolytically conducting solution.
2. An electrolytic recording medium according to claim 1 in which an additional acid is incorporated therewith for pH adjustment.
3. An electrolytic recording medium according to claim 1 in which an acid solution is incorporated therewith, the acidity of the solution being approximately pH 1.25.
4. An electrolytic recording medium according to claim 1 in which an acid solution is incorporated containing at least one compound selected from the group consisting of sulfuric acid, nitric acid, and hydrochloric acid.
5. An electrolytic recording medium according to claim 1 in which a stabilizer is incorporated to prevent discoloration of the recording medium prior to marking and of the background thereof after marking.
6. An electrolytic recording medium according to claim 1 in which a stabilizer is incorporated to prevent discoloration of the recording medium prior to marking and of background thereof after marking and an addi-

- tional acid solution is incorporated for pH adjustment.
7. An electrolytic recording medium according to claim 1 in which thiourea is incorporated as a stabilizer.
  8. An electrolytic recording medium according to claim 1 in which the electrolyte is selected from the group consisting of alkali metal chlorides and alkali metal nitrates.
  9. An electrolytic recording medium according to claim 1 in which the electrolyte is selected from the group consisting of sodium and potassium chlorides, and sodium and potassium nitrates.
  10. An electrolytic recording medium according to claim 1 in which the electrolyte is selected from the group consisting of alkali metal chlorides and alkali metal nitrates, and incorporated in a solution containing at least one compound selected from the group consisting of sulfuric acid, nitric acid, and hydrochloric acid.
  11. An electrolytic recording medium according to claim 1 in which the electrolyte is selected from the group consisting of nitrates and chlorides of sodium and potassium, and there is incorporated an acid solution containing at least one compound selected from the group consisting of sulfuric acid, nitric acid and hydrochloric acid, and thiourea as a stabilizer.
  12. An electrolytic recording medium according to claim 1 in which is included a stabilizer to prevent discoloration of the recording medium prior to marking and of the background thereof after marking and an additional acid for pH adjustment, the impregnant consisting essentially in approximate parts by relative weights of chromotropic acid 2, electrolyte 10, acid 5 as said additional acid, and stabilizer 0.2 as said stabilizer.
  13. An electrolytic recording medium according to claim 1 in which the components are in an aqueous solution and include a stabilizer to prevent discoloration of the recording medium prior to marking and of the background thereof after marking, the solution consisting essentially in approximate parts by relative weight of chromotropic acid 2, sodium chloride 10, 6 N sulfuric acid 5, and thiourea 0.2 as said stabilizer.

40 References Cited in the file of this patent  
UNITED STATES PATENTS

|           |                 |                |
|-----------|-----------------|----------------|
| 2,358,839 | Wagner          | Sept. 26, 1944 |
| 2,419,296 | Solomon         | Apr. 22, 1947  |
| 2,433,632 | Solomon         | Dec. 30, 1947  |
| 2,459,521 | Greig           | Jan. 18, 1949  |
| 2,485,678 | Tripple         | Oct. 25, 1949  |
| 2,541,488 | Vanselow et al. | Feb. 13, 1951  |
| 2,776,252 | Schwartz        | Jan. 1, 1957   |
| 2,864,748 | Mones           | Dec. 16, 1958  |

OTHER REFERENCES

55 Spot Tests Inorganic Reactions, F. Feigl, Elsevier Pub. Co., N.Y. 1954, pages 187 and 188.